

## UNITED STATES PATENT OFFICE.

PHILIP K. FUNKE, OF ALAMEDA, CALIFORNIA.

## CANDLE.

No Drawing.

Application filed January 30, 1925. Serial No. 5,902.

My invention relates to improvements in candles and more especially to that type of candles which burn with a colored flame.

An important object of my invention is to 5 provide a device of the above mentioned character in which the flame is colored to correspond to the odor or perfume that the candle gives off when burning.

Heretofore it has not been possible to color 10 the flames of ordinary candles consisting of paraffin, ceresin, etc., but I have discovered that with the use of inorganic wax, such as paraffin, combined with certain acids, such as stearic and palmitic, in combination with 15 certain chemicals, a candle may be produced that will burn with a colored flame.

I contemplate adding aromatic oils and 20 perfume bases to the candle in the process of manufacture in such manner that odor will be produced without smoke.

These candles will be colored to indicate 25 the odor they will emit while burning, as for example, a candle that would give a lavender odor would be dyed lavender.

I also contemplate coloring the flame of 30 the candle to indicate the odor to be emitted.

I also intend indicating the color of the 35 flame of a candle by dyeing it that color.

For coloring the flame I intend using par- 40 affin mixed with stearic acid agitated with air, which when mixed with certain chemicals will produce colored flames. The several chemicals that will give the candle flame the desired color will be mixed with the inor-

ganic wax in the proper proportions (paraf- 45 fin 75% and stearic acid 25%) or they may be incorporated in a specially prepared wick woven from long staple cotton to hold the chemicals contained in solution in which the

wick will be immersed, and then dried, the 50 wick being larger than the usual wick to permit it to absorb enough of the solution containing the flame coloring chemicals to properly color the flame. In making the candle, the

55 mixture of paraffin 75% and stearic acid 25% is melted, and when cool, but before it hardens, is agitated with compressed air which leaves the mixture light in weight and porous, allowing it to burn rapidly.

To obtain a red candle, red aniline dye is 60 added to the liquid wax stearic acid mixture and one-half of one per cent oil of rose geranium is also added at the same time. To obtain a red flame the wick which has been sat-

65 urated in a solution of 25 parts strontium

nitrate, 15 parts potassium chlorate, 4 parts antimony sulphate, and 13 parts sulphur, is placed in the center of a candle mold and the cooling mixture of paraffin and stearic acid, is then poured into the mold around the wick 60 and cooled rapidly. In order to improve the color of the flame, 2½% of a mixture of the dry chemicals specified above may be added to the paraffin and stearic acid at the time the aniline dye and the rose geranium oil are 65 mixed.

I may use, for example, to obtain a blue 70 colored flame, a combination of potassium nitrate 8 parts, liquid sulphur 4 parts, and copper sulphate 4 parts. The specially prepared wick will be immersed in a solution (10%) of equal parts nitrate of potash and copper sulphate. The chemicals themselves will be mixed with the candle base in sufficient amounts to get the proper color flame 75 for example 2½%, as set out above.

To obtain a red flame I may use strontium 80 nitrate, 25 parts, potassium chlorate, 15 parts, antimony sulphate, 4 parts and sulphur, 13 parts, saturating the wick in a solution (10%) of equal parts strontium nitrate and potassium chlorate.

The chemicals above mixed with the candle 85 base (paraffin and stearic acid) and used for saturating the wicks are for producing the colored flames. The color of the candle itself will be made with aniline dye.

As an example, a candle colored with purple aniline will contain essential oil lavender, 90 which will diffuse odor as the candle is consumed, or a candle will be colored red with aniline and combined with essential oil rose geranium.

These essential oils are very volatile and fragrant, being evaporated as the candle 95 burns. The heat generated by the burning of the candle will vaporize the oils before they can be consumed by the flame because of their volatility and consequently, odor will be produced without smoke.

It is to be understood however that I do not restrict myself to these combinations of chemicals, or colors, but may resort to various changes without departing from the spirit of my invention or the scope of the subjoined claims.

Having described my invention what I claim and desire to protect by Letters Patent is:

1. A candle having an incense incorpo- 110

rated therein, said candle being dyed with a color known by a term which also designates the incense in the candle.

2. A candle of inorganic wax and a fatty acid, said candle having salts incorporated therein to produce a colored flame, said candle being dyed the same color as that adapted to be imparted to the flame by the salts.

3. A candle of inorganic wax and a fatty acid, an incense incorporated in said candle, and salts incorporated in the candle and adapted to impart a color to the flame of the candle, said color being known by a term

which also designates the kind of incense in the candle.

15

4. A candle of inorganic wax and a fatty acid, said candle having an incense incorporated therein, and salts incorporated in said candle and adapted to impart a color to the flame of the candle, said color of the flame being known by a term which also designates the kind of incense in the candle, said candle being dyed the color imparted to the flame by the salts.

In testimony whereof I affix my signature.  
PHILIP K. FUNKE.